

F. J. MAYWALD.  
PROCESS FOR PRODUCING PHOSPHORIC ACID.  
APPLICATION FILED SEPT. 10, 1902.

902,157.

Patented Oct. 27, 1908.



WITNESSES:

M. M. Connor.  
M. Page

INVENTOR

Frederick J. Maywald

BY

H. M. Marber

ATTORNEY

# UNITED STATES PATENT OFFICE.

FREDERICK J. MAYWALD, OF BROOKLYN, NEW YORK.

## PROCESS FOR PRODUCING PHOSPHORIC ACID.

No. 902,157.

Specification of Letters Patent.

Patented Oct. 27, 1908.

Application filed September 10, 1902. Serial No. 122,759.

*To all whom it may concern:*

Be it known that I, FREDERICK J. MAYWALD, a citizen of the United States, residing in Brooklyn, in the county and State of New York, have invented a Process of Producing Phosphoric Acid; and I do hereby declare the following to be a full, clear, and exact description of the invention, such as will enable others skilled in the art to which it 10 appertains to make and use the same.

My invention relates to a process of producing phosphoric acid from natural phosphates, such as are known as phosphate rock, and is applicable to aluminum phosphate, 15 calcium phosphate, and mixtures of calcium and aluminum phosphates and calcium, aluminum and iron phosphates. These phosphates having an earthy base of alkaline earth or earthy oxid are all relatively 20 infusible.

The process consists in passing an electric current through a mass of the comminuted material, and collecting the fumes evolved, preferably by condensing them to a powder, 25 which is readily soluble in water. Under the conditions of operation, as hereinafter set forth, the phosphate simply dissociates and the  $P_2O_5$  distils away, leaving a residue of base or basic phosphate. The  $P_2O_5$  is 30 collected as such.

The objects of my invention are, to produce phosphoric acid in a simple and inexpensive manner and in a readily soluble form.

35 In the drawings which accompany and form a part of this specification, I illustrate diagrammatically an apparatus which may be used for carrying out my process.

Said apparatus consists of a crucible 1, 40 which may be of plumbago or graphite or other suitable material, and may be provided at its bottom with an aperture through which may be inserted a carbon electrode 2. Above this crucible is a condensing hood 3 45 for collecting the fumes evolved and in said hood is an aperture through which may be inserted another carbon electrode 4. The hood may be constructed of metal and if radiation to the surrounding atmosphere is 50 not sufficient to keep it cool, it may be cooled artificially, as by blowing a blast of air upon it.

A dynamo or other generator 5 is placed in circuit with the carbon electrodes 2 and 55 4, and in this circuit there may be an adjustable resistance 6.

In carrying out the process, the material to be used is placed, preferably in a finely pulverized condition, within the crucible, retort, furnace or other object within which the process is conducted. A trace of carbon in the material will often aid in the evolution of the phosphoric acid if the material be difficult to dissociate. But the addition of carbon is not ordinarily necessary. I 65 ordinarily employ a current of from 40 to 60 volts. The voltage is higher at the beginning of the operation, but as the mass becomes hot the voltage will fall of itself.

It is preferable to employ a short arc, the 70 carbon electrodes being placed close together, as there is then less tendency to produce phosphorus than when a long arc is used. But I have found resistance heating to be effective; the resistance heating being effected 75 by separating the carbons when the mass within the crucible is hot, so that no distinct arc is produced but the electric current permeates the mass of granular material between the two electrodes. In any case, the 80 temperature of the mass is kept below the melting point thereof, as I have found that if the mass be heated to the melting point it is impracticable to drive off all of the phosphoric acid. But when not heated to 85 the melting point, the mass remains in a porous condition, which permits free escape of phosphoric acid.

A slight amount of air may be permitted 90 to enter the crucible or furnace to oxidize any phosphorus that may be formed. Such air may be introduced through a slight space left between the crucible and condensing hood or by other suitable means.

The result of the passage of the electric 95 current is to dissociate the phosphate and liberate the phosphoric acid in anhydrous form from the material treated, and the fumes of this anhydrous acid or  $P_2O_5$  condense upon the hood 3 as a powder which 100 is readily soluble in cold water. From time to time the hood 3 may be removed and the powder which thus collects dislodged therefrom.

I do not limit myself to the use of the particular apparatus shown in the drawings, or to the use of any particular apparatus, or to any particular material from which to form the crucible or furnace, or the electrodes, or the condensing hood; nor do I 110 limit myself to any particular form of condensing apparatus, nor to any particular

strength of current. Likewise, the process may be applied to the extraction of phosphoric acid from other salts of said acid than are above specified.

Having thus completely described my invention, what I claim and desire to secure by Letters Patent is:

1. The process of treating phosphates which consists in producing a low potential arc in a granular mass of phosphates having an earthy base and heating such phosphates to a dissociating temperature, thereby decomposing the same into phosphoric oxid and base, and in collecting the fumes of phosphoric oxid as such.

2. The process of treating phosphates which consists in subjecting a granular mass of phosphates having an earthy base to heat and the action of a short electric arc and heating such phosphates to a dissociating temperature, thereby decomposing the same into phosphoric oxid and a basic residue, and in collecting evolved fumes of phosphoric oxid.

3. The process of treating phosphates which consists in subjecting a granular mass of relatively infusible phosphates to heat and the action of a short electric are while permitting access of air to such mass, and heating such phosphates to a dissociating temperature, thereby decomposing said phosphates into phosphoric oxid and a basic resi-

due, and in collecting the evolved fumes of phosphoric oxid.

4. The process of treating phosphates 35 which consists in subjecting a granular mass of relatively infusible phosphates to the action of the arc produced by an electric current not materially exceeding 60 volts in potential, and heating such phosphates to a 40 dissociating temperature, thereby decomposing said phosphates into phosphoric oxid and a basic residue, and in collecting the fumes of phosphoric oxid produced.

5. The process of treating phosphates 45 which consists in initially heating a granular mass of relatively infusible phosphates by means of a short electric arc produced by an electric current not materially exceeding 60 volts in potential, continuing the 50 heating by passing a low potential current through said granular mass and heating such phosphates to a dissociating temperature thereby decomposing the same into phosphoric oxid and a basic residue, and in 55 collecting the fumes of phosphoric oxid produced.

In testimony whereof I affix my signature, in the presence of two witnesses.

FREDERICK J. MAYWALD.

Witnesses:

H. M. MARBLE,  
A. H. PERLES.